# EUROPEAN PATENT SPECIFICATION

(11) **EP 0 674 221 B1**
(45) Date of publication and mention of the grant of the patent: **26.08.1998**
(21) Application number: 95200377.0
(22) Date of filing: 16.02.1995
(51) Int. Cl.: G03C 7/388

(54) **Surfactants and hydrophilic colloid compositions and materials containing them**
Tenside und hydrophile, kolloidale Zusammensetzungen und diese enthaltenden Materialien
Agents tensioactifs et compositions colloidales hydrophiles et matériaux les contenant

(30) Priority: 18.02.1994 US 198729; 19.02.1994 GB 9403209
(43) Date of publication of application: 27.09.1995
(73) Proprietor: KODAK LIMITED, Harrow, Middlesex HA1 4TY (GB); EASTMAN KODAK COMPANY, Rochester, New York 14650-2201 (US)
(72) Inventor: Pitt, Alan Robert, Harrow, Middlesex HA1 4TY (GB); Caesar, Julian Claudius, Harrow, Middlesex HA1 4TY (GB); Gibson, Danuta, Harrow, Middlesex HA1 4TY (GB); Wear, Trevor John, Harrow, Middlesex HA1 4TY (GB); Young, David John, Harrow, Middlesex HA1 4TY (GB); King, Scott, c/o EASTMAN KODAK CO., Rochester, New York 14650-2201 (US)
(74) Representative: Nunney, Ronald Frederick Adolphe

(56) References cited:
- EP-A- 0 560 457
- WO-A-93/03420
- RESEARCH DISCLOSURE, vol. 308, no.119, 10 December 1989 EMSWORTH, GB, ANONYMOUS 'Photographic silver halide materials - and their additives processing and systems'

## Description

### Field of Invention

The invention relates to surfactants and their use as dispersing aids in the preparation of hydrophilic colloid compositions having hydrophobic particles dispersed therein. Such compositions may be used in the preparation of multilayer photographic materials.

### Background of the Invention

A wide variety of surfactants have been described for use in the preparation of photographic materials.

JP56-19042 describes various diester sulfoitaconates as dispersing aids for photographic additives. The two ester linked hydrophobic groups include a number of substituted or unsubstituted alkyl or aryl groups.

US-A-3 948 663 describes photographic materials containing certain sulfosuccinate surface active agents and refers to their possible use as dispersing aids and coating aids. A specific example of such a surface active agent is sodium dioctyl sulfosuccinate which is commercially available as Aerosol™OT.

WO93/03420 describes a method of making fine particle photographic coupler dispersions which comprises forming a dispersion of photographic coupler, coupler solvent and auxiliary coupler solvent in an aqueous gelatin medium containing at least about 1% by weight of an anionic surfactant having a hydrophobicity of 2-10 log P(OH) and washing the dispersion with water for a time sufficient to remove at least one fourth of the surfactant. Anionic surfactants of diverse structures may be employed and included among several named surfactants is diphenylbutyl sodium sulfosuccinate.

A shortcoming of the use of surfactants described in JP56-19042 and US-A-3 948 663 is the very low surface tension values exhibited by the compounds at concentrations above their critical micelle concentration (CMC). In the simultaneous multilayer coating of hydrophilic colloid layers, it is essential that the surface tension of the top layer is lower than that of any of the underlying layers if it is to remain spread during the coating operation. If one of the underlying layers has a lower surface tension than the top layer it drives the top layer in from the edges towards the centre of the coating. This is often termed "edge retraction". The larger the surface tension imbalance, the more disruptive is the effect. Large differences can cause retraction of the whole coating pack and general layer inversions. The surface tension of underlying layers in the multilayer coating of photographic materials is often dominated by the surfactant dispersing aid that is used to stabilize the emulsified hydrophobic particles therein e.g. colour couplers and their associated solvents.

When such prior art surfactants are used as dispersing aids for emulsified materials that are incorporated in underlying hydrophilic colloid layers during simultaneous multilayer coating, a constraint is put on the choice of surfactant or surfactant concentration required for the overlying layers i.e. coating latitude is relatively narrow.

Another shortcoming of the use of the surfactants described in JP56-19042 and US-A-3 948 663 as dispersing aids for photographic couplers in hydrophilic colloid compositions is that the photographic properties of such compositions e.g. the liquid dispersion reactivity, can be less than desired.

A further shortcoming of the use of the surfactants described in JP56-19042 and US-A-3 948 663 as dispersing aids in photographic materials is that they can contribute to foaming during photographic processing, especially in seasoned developers where surfactants have leached out from the material and have built up in concentration.

### Problem to be Solved by the Invention

The invention overcomes the coating latitude problem associated with the prior art dipersing aids.

Limitations in the photographic properties of dispersions of photographic couplers in hydrophilic colloids can be overcome.

The invention can reduce the foaming which can occur during the processing of photographic materials containing the prior art dispersing aids.

### Summary of the Invention

The invention provides a method of preparing a multilayer photographic material which comprises
(a) simultaneously coating on a support a plurality of aqueous hydrophilic colloid layers including at least one light-sensitive silver halide emulsion layer wherein at least one of the underlying hydrophilic colloid layers contains hydrophobic particles dispersed therein with the aid of a surfactant and,
(b) drying the coated layers, characterised in that the surfactant has the structure wherein
   R is H or methyl provided that when each n=1, each R is methyl;
   M is a cation; and,
   n is an integer from 1 to 6;

Also provided is use of a surfactant having the structure I in the method described above as an agent which improves coating latitude.

In another aspect, the invention relates to use of a surfactant having the structure I in a multilayer photographic material comprising a support bearing a plurality of hydrophilic colloid layers including at least one light-sensitive silver halide emulsion layer wherein at least one of the underlying hydrophilic colloid layers contains hydrophobic particles dispersed therein with the aid of the surfactant; in order to reduce the foaming which can occur during photographic processing of the material.

The invention also provides a method of preparing a composition comprising a hydrophilic colloid having hydrophobic particles dispersed therein comprising dispersing a hydrophobic material comprising a photographic coupler into an aqueous solution of a hydrophilic colloid in the presence of the surface active agent characterised in that the surfactant has the structure I and the surfactant is used in an amount less than 1 weight percent without a washing step to remove at least one fourth of the surfactant.

### Advantageous Effect of the Invention

By providing aqueous hydrophilic colloid melts with high surface tension minima, the invention enables increased coating latitude.

Improved photographic performance can be achieved with dispersions of a photographic coupler in a hydrophilic colloid. The nature of the improvement depends on the type of coupler dispersion. For example, with a microprecipitated dispersion, the benefits include decreased droplet size, increased liquid dispersion reactivity, and increased Dmax in coated product. With a homogenized dispersion, the benefits include increased liquid dispersion reactivity, and increased shoulder density and contrast in coated product.

Another advantage is reduced foam formation during photographic processing, especially in seasoned developer.

### Detailed Description of the Invention

In structure I, the cation M is a positively charged atom or group of atoms preferably chosen from alkali metal cations e.g. Na⁺, or ammonium.

Preferred compounds include those wherein each n is from 2 to 4, and each R is H. In a particularly preferred compound, each n is 3, and each R is H.

The compounds may be water soluble or water dispersible.

The compounds may be prepared by the esterification of maleic acid with a phenylalkanol wherein the alkanol has from 3 to 8 carbon atoms. A specific method which can be used in respect of all the compounds is given below in Example 1.

Compositions comprising a hydrophilic colloid having hydrophobic particles dispersed therein may be formed by a process comprising dispersing a hydrophobic material into an aqueous solution of a hydrophilic colloid in the presence of the surface active agent.

For homogenized dispersions, the surface active agent is used preferably in an amount from 0.4 to 1.2 , more preferably from 0.6 to 0.9 weight percent based on the weight of the aqueous dispersion.

For microprecipitated dispersions, the surface active agent is used preferably in an amount that provides a molar ratio of surface active agent: hydrophobic material e.g. photographic coupler which is from 1:4 to 2:1.

Regardless of the particular method of preparation, dispersions can be made in accordance with the invention which avoid the coating latitude problems associated with the prior art by using less than about 1 weight percent of the surfactant and without requiring a washing step to remove at least one fourth of the surfactant e.g. no washing step is used.

The invention is particularly useful in the preparation of photographic compositions and materials.

In the following discussion of suitable materials for use in the compositions and materials of this invention, reference will be made to Research Disclosure, December, 1989, Item 308119, published by Kenneth Mason Publications, Ltd., Dudley Annex, 12a North Street, Emsworth, Hampshire, P010 7DQ, UK. This publication will be identified hereafter by the term Research Disclosure.

A number of hydrophobic photographic additives used in light sensitive photographic materials are oil-soluble and are used by dissolving them in a substantially water-insoluble, high boiling point solvent which is then dispersed in an aqueous hydrophilic colloid solution with the assistance of a dispersing aid. Such oil-soluble additives include image forming dye couplers, dye stabilizers, antioxidants and ultra-violet radiation absorbing agents. A typical solvent used to dissolve the additive is aromatic e.g. di-n-butyl phthalate.

Gelatin is the preferred hydrophilic colloid, but other hydrophilic colloids can be used alone or in combination with gelatin.

Suitable methods of preparing photographic dispersions are described in Research Disclosure, Sections XIV A and XIV B. For example, homogenised oil in aqueous gelatin dispersions of photographic couplers can be prepared by dissolving the coupler in a coupler solvent and mechanically dispersing the resulting solution in an aqueous gelatin solution (see U.S. Patent No. 2,322,027).

Alternatively, microprecipitated dispersions of photographic couplers prepared by solvent and/or pH shift techniques are becoming more widely used (see references: U.K. Patent No. 1,193,349; Research Disclosure 16468, Dec 1977 pp 75-80; U.S. Serial No. 288,922 (1988) by K.Chari; U.S. Patent Nos. 4,970,139 & 5,089,380 by P.Bagchi; U.S. Patent No.5,008,179 by K.Chari, W.A.Bowman & B.Thomas; U.S. Patent No. 5,104,776 by P.Bagchi & S.J.Sargeant) and offer benefits in decreased droplet size and often increased reactivity relative to conventional oil-in-water homogenised dispersions.

Multilayer photographic materials according to the invention comprise one or more underlying layers formed from such compositions.

Preferred multilayer photographic materials include color materials of the type described in Research Disclosure, Sections VII A to VII K.

Methods of preparing multilayer photographic materials by simultaneously coating the layers are known. Particular methods are described in Research Disclosure, Sections XV A and XV B. Such methods include extrusion coating and curtain coating.

The hydrophobic material dispersed in the hydrophilic colloid may be a photographic coupler.

Couplers which form cyan dyes upon reaction with oxidized color-developing agents are described in such representative patents and publications as U.S. Patent Nos. 2,772,162; 2,895,826; 3,002,836; 3,034,892; 2,747,293; 2,423,730; 2,367,531; 3,041,236; and 4,333,999; and Research Disclosure, Section VII D.

Couplers which form magenta dyes upon reaction with oxidized color developing agents are described in such representative patents and publications as: U.S. Patent Nos. 2,600,788; 2,369,489; 2,343,703; 2,311,082; 3,152,896; 3,519,429; 3,062,653; and 2,908,573; and Research Disclosure, Section VII D.

Couplers which form yellow dyes upon reaction with oxidized and color developing agents are described in such representative patents and publications as: U.S. Patent Nos. 2,875,057; 2,407,210; 3,265,506; 2,298,443; 3,048,194; and 3,447,928; and Research Disclosures, Section VII D.

Couplers which form colorless products upon reaction with oxidized color developing agents are described in such representative patents as: UK Patent No. 861,138; U.S. Patent Nos. 3,632,345; 3,928,041; 3,958,993; and 3,961,959.

The couplers can be dissolved in a solvent and then dispersed in a hydrophilic colloid. Examples of solvents usable for this process include organic solvents having a high boiling point, such as alkyl esters of phthalic acid (for example, dibutyl phthalate, dioctyl phthalate), phosphoric acid esters (for example, diphenyl phosphate, triphenyl phosphate, tricresyl phosphate, dioctyl butyl phosphate) citric acid esters (for example, tributyl acetyl citrate) benzoic acid esters (for example, octyl benzoate), alkylamides (for example, diethyl laurylamides), esters of fatty acids (for example dibutoxyethyl succinate, dioctyl azelate), trimesic acid esters (for example, tributyl trimesate); and organic solvents having a boiling point of from about 30° to about 150°C., such as lower alkyl acetates (for example, ethyl acetate, butyl acetate), ethyl propionate, secondary butyl alcohol, methyl isobutyl ketone, b-ethoxyethyl acetate, methyl cellosolve acetate. Mixtures of organic solvents having a high boiling point and organic solvents having a low boiling point can also be used.

As the binder or the protective colloid for the photographic emulsion layers or intermediate layers of the photographic light-sensitive material of the present invention, gelatin is advantageously used, but other hydrophilic colloids can be used alone or together with gelatin.

As gelatin in the present invention, not only lime-processed gelatin, but also acid-processed gelatin may be employed. The methods for preparation of gelatin are described in greater detail in Ather Veis, *The Macromolecular Chemistry of Gelatin,* Academic Press (1964).

As the above-described hydrophilic colloids other than gelatin, it is possible to use proteins such as gelatin derivatives, graft polymers of gelatin and other polymers, albumin, casein; saccharides such as cellulose derivatives such as hydroxyethyl cellulose, cellulose sulfate, sodium alginate, starch derivatives; and various synthetic hydrophilic high molecular weight substances such as homopolymers or copolymers, for example, polyvinyl alcohol, polyvinyl alcohol semiacetal, poly-N-vinylpyrrolidone, polyacrylic acid, polymethacrylic acid, polyacrylamide, polyvinyl imidazole, polyvinylpyrazole.

In the photographic emulsion layers or other hydrophilic colloid layers of the photographic light-sensitive material of the present invention can be incorporated various surface active agents as coating aids or for other various purposes, for example, prevention of charging, improvement of slipping properties, acceleration of emulsification and dispersion, prevention of adhesion and improvement of photographic characteristics (for example, development acceleration, high contrast, and sensitization).

Surface active agents which can be used are nonionic surface active agents, for example, saponin (steroid-based), alkyene oxide derivatives (for example, polyethylene glycol, a polyethylene glycol/polypropylene glycol condensate, polyethylene glycol alkyl ethers or polyethylene glycol alkylaryl ethers, polyethylene glycol esters, polyethylene glycol sorbitan esters, polyalkylene glycol alkylamines or polyalkylene glycol alkylamides, and silicone/polyethylene oxide adducts, and the like), glycidol derivatives (for example, alkenylsuccinic acid polyglyceride and alkylphenol polyglyceride), fatty acid esters of polyhydric alcohols and alkyl esters of sugar; anionic surface active agents containing an acidic group, such as a carboxy group, a sulfo group, a phospho group, a sulfuric acid esters group, and a phosphoric acid ester group, for example, alkylcarboxylic acid salts, alkylsulfonic acid salts, alkylbenzenesulfonic acid salts, alkylnaphthalenesulfonic acid salts, alkylsulfuric acid esters, alkylphosphoric acid esters, N-acyl-N-alkyltaurines, sulfosuccinic acid esters, sulfoalkylpolyoxyethylene alkylphenyl ethers, and polyoxyethylene alkylphosphoric acid esters; amphoteric surface active agents, such as amino acids, aminoalkylsulfonic acids, aminoalkylsulfuric acid or aminoalkylphosphoric acid esters, alkylbetaines, and amine oxides; and cationic surface active agents, for example, alkylamine salts, aliphatic or aromatic quaternary ammonium salts, heterocyclic quaternary ammonium salts (for example, pyridinium and imidazolium) and aliphatic or heterocyclic phosphonium or sulfonium salts.

In the photographic emulsion layer of the photographic light-sensitive material used in the present invention, any of silver bromide, silver iodobromide, silver iodochlorobromide, silver chlorobromide and silver chloride may be used as the silver halide.

The light-sensitive silver halide contained in the photographic material can be processed following exposure to form a visible image by associating the silver halide with an aqueous alkaline medium in the presence of a developing agent contained in the medium or the material. Suitable types of photographic processing are described in Research Disclosures, Section XIX A to XIX J. Suitable developing agents are described in Research Disclosures, Section XX A to XX B.

The following Examples further illustrate the invention.

A number of compounds referred to in the Examples are as follows:

### Example 1

### Synthesis of sodium di(4-phenylbut-1-yl)sulfosuccinate

All sodium sulfosuccinate surfactants were prepared following the general method outlined below: A solution of maleic anhydride (32.6g,0.33mol), 4-phenyl-1-butanol (100.0g,0.66mol) and concentrated sulfuric acid (1.5cm³) was suspended in toluene (750cm³) and refluxed for 16 hours in a flask equipped with a Dean and Stark trap. On cooling, the toluene solution was reduced to 1/4 volume at reduced pressure on a rotary evaporator and washed with saturated sodium hydrogen carbonate(2x200cm³) and then with water (2x200cm³). The organic layer was dried over magnesium sulfate and the solvent removed at reduced pressure (15 mmHg, 50°C) to give an intermediate diester as a clear oil (119.5g, 95%).

A solution of sodium metabisulfite (65.7g, 0.34mol) in water (400cm³) was added to a solution of this diester (119.5g, 0.31mol) in ethanol (400cm³) and the mixture brought to reflux over 15 minutes. Sodium sulfite (36.0g, 0.28mol) was then added portionwise to the mixture over 40 minutes and the reaction then allowed to reflux overnight for convenience. The reaction mixture was evaporated to dryness (15mm Hg,50°C) and then extracted into ethyl acetate (1.5L, hot) and filtered. The ethyl acetate solution was concentrated and allowed to cool to give the product as a white crystalline solid (139.8g, step yield 93%, overall yield 87%).

Spectroscopic and 1 Hnmr data was consistent with the proposed product, sodium di(4-phenylbut-1-yl)sulfosuccinate.

### Example 2

Tables IA and IB compare the surface tension data of the compounds of the invention with commercial examples of dialkyl sulfosuccinate, Aerosol™MA (sodium dihexyl sulfosuccinate), Aerosol™OT (sodium diisooctyl sulfosuccinate) and Aerosol™AY (sodium dipentyl sulfosuccinate). The method used for surface tension measurements is as follows.

The measurement of surface tension of an aqueous solution containing surfactant was measured over a concentration range including the critical micelle concentration using the Wilhelmy technique (Padday, J.F., 2nd Int. Congress of Surface Activity, I, 1, 1957) with a platinum blade. Comparative dynamic surface tension measurements were also determined by the same technique using an overflowing circular weir (ibid.). The average surface age of the solutions in the overflowing weir has been estimated to be of the order of 0.1 seconds.

**TABLE IA:**

| **Surface Tension (mN/m) of Solutions in Water at 25°C** | | | | |
|---|---|---|---|---|
| Compounds Tested Invention | Concentration wt% in Water | | | CMC |
| | 0.25% | 0.5% | 1.0% | wt% |
| n=2, R=Me | 44.9 | 40.3 | 39.0 | 0.64 |
| n=2, R=H | 37.6 | 37.6 | 37.9 | 0.23 |
| n=3, R=H | 42.1 | 41.7 | 40.2 | 0.10 |
| n=4, R=H | - | - | 37.5 | - |

**TABLE IB:**

| **Surface Tension (mN/m) of Solutions in Water at 25°C (Trade Literature)** | | | | |
|---|---|---|---|---|
| Compounds Tested Comparisons | Concentration wt% in Water | | | CMC |
| | 0.25% | 0.5% | 1.0% | wt% |
| Aerosol OT | 27.5 | 26.0 | 26.0 | ∼0.07 |
| Aerosol MA | 38.2 | 30.8 | 27.8 | 0.6-0.7 |
| Aerosol AY | 41.6 | 35.2 | 29.2 | 0.9-1.2 |

Tables IA and IB show clearly that once the concentrations of the surfactants approach or go beyond their CMC where surface tension values tend to plateau, the compounds of this invention exhibit much higher values of surface tension than the corresponding dialkyl equivalents. Equivalents denote compounds of similar CMC. On comparing equivalent compounds at such concentrations, the materials of this invention show surface tension values that are 10-14 mN/m higher.

Tables IIA and IIB show similar data to Tables IA and IB, but the measurements were conducted in solutions containing 7% deionised Type IV bone gelatin in water at 40°C to simulate a coating melt.

**TABLE IIA:**

| **Surface Tension (mN/m) of Solutions in 7% Deionised Type IV Bone Gelatin Water at 40°C. (Compounds of This Invention)** | | | | |
|---|---|---|---|---|
| Compounds Tested Invention | Wt% Concentration in 7% Deionised Gelatin Solution | | | CMC |
| | 0.03% | 0.10% | 0.30% | wt% |
| n=2, R=Me | 49.4 | 44.9 | 41.8 | ∼0.3 |
| n=2, R=H | 49.5 | 44.2 | 43.3 | ∼0.1 |
| n=3, R=H | 43.2 | 42.8 | 42.8 | ∼0.03 |
| n=4, R=H | 42.1 | 41.7 | 40.7 | ∼0.01 |

In the following Table, the comparison compounds are sulfosuccinates having the formula

**TABLE IIB:**

| **Surface Tension (mN/m) of Solutions in 7% Deionised Type IV Bone Gelatin Water at 40°C (Comparison Compounds)** | | | | |
|---|---|---|---|---|
| Compounds Tested Comparisons | Wt% Concentration in 7% Deionised Gelatin solution | | | CMC |
| | 0.03% | 0.10% | 0.30% | wt% |
| Aerosol OT | 29.2 | 28.9 | 28.7 | ∼0.01 |
| Aerosol MA | 41.9 | 36.3 | 31.4 | ∼0.1 |
| R¹=n-hexyl | 37.0 | 32.0 | 30.0 | ∼0.1 |
| R¹=n-pentyl | 46.0 | 39.9 | 34.4 | ∼1.3 |

Tables IIA and IIB also show clearly that once the concentrations of the surfactants approach or go beyond their CMC in aqueous gelatin solution, the compounds of this invention still exhibit much higher values of surface tension than the corresponding dialkyl equivalents. On comparing equivalent compounds at such concentrations, the materials of this invention again show surface tension values that are 10-14 mN/m higher.

In general therefore, the materials of this invention offer the advantage of relatively high surface tension minima coupled with reasonably low CMCs (up to 0.3 weight % in 7% gelatin in water) in situations where low values are undesirable, e.g. in underlying layers during simultaneous multilayer coating.

### Example 3

**Increased Coating Latitude Using Materials of Invention as Dispersing Aid in Underlying Layers during Simultaneous Multilayer Coating:**

To show that the compounds of this invention permit a wider coating latitude when used as dispersing aids in the underlying layer of a simultaneous two layer coating, the following format was coated at 15 m/min at 40°C with a range of different surfactants:

| | |
|---|---|
| TOP LAYER coated at 10.8ml/m² (1ml/ft²) | 10% type IV regular bone gelatin containing 0.3 wt% surfactant and a blue dye marker. |
| BOTTOM LAYER coated at 59ml/m² (5.5ml/ft²) | coupler dispersion (coupler I or II) diluted to 4% gelatin by weight with water containing a red dye marker. |
| 12.7cm (5ins) wide polyethylene terephthalate film base (suitably subbed to give good adhesion to gelatin) | |

### Bottom layer:

A dispersion of a colour coupler was made according to the following recipes:

### 2 kg Dispersion of Coupler I:

258g of coupler I was dissolved in a mixture of 65g di-n-butyl phthalate and 65g of solvent III at 145°C to make Solution A. 176g of gelatin was dissolved in 1354g of water containing 17.6g of dispersing aid (surfactant under test) and 31g of propionic acid/sodium proprionate preservative to make Solution B. After heating Solution B to 80°C, solution A was added to Solution B and the whole mixture was immediately homogenised for 5 minutes at 10,000 rpm with a Kinematica Polytron homogeniser fitted a 35mm diameter head.

### 1.7 kg Dispersion of Coupler II:

149g of coupler II was dissolved in a mixture of 58.5g di-n-butyl phthalate, 22.3g of solvent III, 79.1g of stabiliser IV and 14.9g of scavenger V at 145°C to make Solution C. 149g of gelatin was dissolved in 1180g of water containing 16.4g of dispersing aid (surfactant under test) and 32.7g of propionic acid/sodium propionate preservative to make Solution D. After heating Solution D to 80°C, solution C was added to Solution D and the whole mixture was immediately homogenised for 5 minutes at 10,000 rpm with a Kinematica Polytron homogeniser fitted with a 35mm diameter head.

The coupler dispersion, which contained approximately 9% gelatin by weight, was then diluted at 40°C to a gelatin content of 4 wt% with water which contained a red dye marker. The resulting mixture was used for the bottom layer of a two layer hopper coating as illustrated above.

Thus a range of bottom layer coating melts were made which differed in the dispersion component, the major difference being the dispersing aid (surfactant) used. The main objective was to compare four diarylalkyl sulfosuccinate dispersing aids of this invention with two commercial dialkyl sulfosuccinate dispersing aids and the commercial surfactant Alkanol™XC (sodium triisopropyl naphthalene sulphonate). Two types of coupler, I and II, were used for making the coupler dispersions. It should be noted for each coupler used that the comparisons of surfactants were between compounds of similar hydrophilic-lipophilic balance, i.e. of similar CMC.

### Top Layer:

Four different surfactants were selected for the top layer coating aid to produce a range of characteristic values of minimum surface tension, 25.5 -37.2mN/m. A working concentration of 0.3% was chosen to ensure that the surfactants were being used well beyond their CMC in order that the surface tensions of their respective solutions under dynamic conditions were very similar to those under static conditions and therefore essentially at a characteristic plateau value. The method used for estimating a dynamic value of surface tension is described Example 2. The materials chosen are listed in the following table together with representative surface tension data.

**TABLE III:**

| **Surface Tension Data** | | |
|---|---|---|
| Surfactant (0.3 wt% Concentration in 7% by wt Type IV Bone Gelatin in Water + Blue Dye | Dynamic Surface Tension | Static Surface Tension |
| | mN/m | mN/m |
| Aerosol OT (AOT) | 25.5 | 25.5 |
| Triton X-100 (TX100) | 30.5 | 30.2 |
| Texofor FN15 (TFN15) | 34.7 | 34.4 |
| SDS | 37.3 | 37.2 |
| Triton™X100 is t-octylphenyl polyethyleneoxide (9.5 moles). | | |
| Texofor™FN15 is nonylphenyl polyethyleneoxide (15 moles). | | |
| SDS is sodium dodecyl sulphate. | | |

A complete 4 X 7 matrix of two layer coatings were made, coating the four types of top layer over the seven types of bottom layer. The dried coatings were then examined to determine whether the top layer had coated successfully over the underlying layer. The coating was deemed successful (OK) if the blue top layer had remained satisfactorily spread over the full width of the coating, and deemed unsuccessful if the bottom layer had caused the top layer to retract from either the edges or if there was multi-cratering in the middle of the coating due to the bottom layer pushing through to the surface. With the red dye in the lower layer and the blue dye in the upper layer, it was extremely clear when the coating was unsuccessful. Table IV summarises the coating results taken from representative strips:

**TABLE IV:**

| **Coating Results - Different Surfactants in Top Layer** | | | | |
|---|---|---|---|---|
| | Top Layer Surfactant | | | |
| Dispersing Aid used: (in bottom layer dispersion component) | AOT Surface Tension 25.5mN/m | TX100 Surface Tension 30.5mN/m | TFN15 Surface Tension 34.7mN/m | SDS Surface Tension 37.3mN/m |
| n=2,R=Me (using coupler I) | OK | OK | OK | OK |
| | | | | |
| n=2,R=H (using coupler I) | OK | OK | Slight fine multiple cratering | Slight edge retraction 1-2 craters |
| | | | | |
| n=3,R=H (using coupler II) | OK | OK | OK | OK |
| | | | | |
| n=4,R=H (using coupler II) | OK | OK | OK | OK |
| Aerosol MA (using coupler I) | OK | Slight edge retraction 40x8mm large crater | Severe retraction of both layers and multiple cratering | Total retraction of top layer into fine stripes |
| | | | | |
| Aerosol OT (using coupler II) | OK | Severe retraction of both layers and multiple large cratering | Severe retraction of both layers and multiple large cratering | Total retraction of top layer and >50% retraction of bottom layer |
| | | | | |
| Alkanol XC (using coupler II) | OK | OK | 3-4mm of edge retraction plus longitudinal break-through and cratering | Severe retraction of both layers and large cratering |

The above results from the two layer coatings clearly show that there is a large increase in coating latitude when the surfactants of this invention are used as the dispersing aids for dispersions in underlying layers during multi-layer coating relative to the comparison compounds. As previously explained and demonstrated here, this means the use of the dispersing aids of this invention puts less constraint upon the choice of surfactant coating aid required in the top layer for good coating. Logically therefore, there should also be less constraint upon the concentration of a coating aid required to give good coating. This aspect is demonstrated in Table V where Aerosol™OT was used as the coating aid in the top layer over a range of concentrations, using the same coating conditions as before.

**Table V.**

| **Coating Results - Different Concentrations of Coating Aid AOT in Top Layer** | | | | |
|---|---|---|---|---|
| Dispersing Aid used: (in bottom layer dispersion component) | Top Layer Surfactant | | | |
| | AOT Concentration 0.02% | AOT Concentration 0.03% | AOT Concentration 0.05% | AOT Concentration 0.07% |
| Invention | | | | |
| n=2,R=H (using coupler I) | OK | OK | OK | OK |
| | | | | |
| n=3,R=H (using coupler II) | OK | OK | OK | OK |

| Comparison Compounds | | | | |
|---|---|---|---|---|
| Aerosol MA (using coupler I) | Retraction from edges and longitudinal break-through of bottom layer | Retraction from edges and longitidunal break-through of bottom layer | OK | OK |
| | | | | |
| Aerosol OT (using coupler II) | Retraction of both layers and multiple cratering | Edge retraction and multiple longtidinal coating breaks | Slight edge retraction of top layer | Very slight edge retraction of top layer |

### Example 4

### Photographic Benefits with Microprecipitated Dispersions

### Increased dispersion reactivity.

Microprecipitated dispersions of photographic couplers, prepared by solvent and/or pH shift techniques are becoming more widely used and offer benefits in decreased droplet size and often increased reactivity relative to conventional oil-in-water homogenised dispersions. When microprecipitated dispersions are prepared using the compounds of this invention, these benefits are increased.

The microprecipitated dispersions were made according to the following method:

The coupler (20g) was dissolved in a mixture of propan-1-ol (40g) and 20% sodium hydroxide solution (5g) at 60°C and poured into a solution of surfactant (weight equimolar with coupler) and polyvinylpyrrolidone (10g) in water (600g). The resulting micellar solution was reduced to pH 6.0 by the dropwise addition of 15% propanoic acid, to form the crude microprecipitated dispersion which was then dialysed through Amicon hollow fibre ultrafiltration cartridges and concentrated to a fifth of its volume.

The liquid dispersion reactivity measurements were made according to the following method. Particle size was measured by photon correlation spectroscopy.

The method used is similar to that described by Bagchi in U.S Patent Nos: 4,970,139; 5,089,380 and 5,104,776. A sample of the dispersion was mixed with a developer solution which contained sodium sulphite, CD-3 developer and EDTA. This was mixed with an activator solution which contained the oxidant sodium persulfate, and a buffer of sodium carbonate and sodium bicarbonate, which brought the pH of the final solution to 10.1 (close to that of processing solutions). The concentrations of oxidant and coupler are much greater than that of the developer. The effect of this is that the oxidant generates oxidised developer which then reacts with the coupler (or with the competing sulfite) to form image dye and side products. The optical density of the dye was then read spectrophotometrically so that for a known dye extinction coefficient, the concentration of the dye could be derived.

If the coupling reaction is treated as a homogeneous, single phase reaction the kinetics of the coupling reaction can be calculated. The coupling reaction and the competing reaction of sulphite with oxidised developer are both assumed to be second order. Remembering that coupler and oxidant concentrations are greater than that of developer, the following expression is derived for the rate constant of the coupling reaction, k₁ which is used as a measure of liquid dispersion reactivity:${\text{k}}_{\text{1}} {\text{= k}}_{\text{2}} \text{ln[a/(a-x)]/ln[b/(b-c+x)]}$ where k₂ is the sulfonation rate constant (previously calculated), a is the coupler concentration, b is the sulfite concentration, c is the developer concentration and x is the concentration of dye.

**TABLE VI.**

| **Microprecipitated dispersions of Coupler VI data.** | | | |
|---|---|---|---|
| SURFACTANT (dispersing aid) | Liquid Dispersion Reactivity | Mean Particle Diameter (nm) | Comment |
| SDS | 9545 | 20.3 | comparison |
| SDBS | 5200 | 25.8 | " |
| Aerosol OT | 4500 | 66.0 | " |
| Aerosol MA | 4575 | 21.6 | " |
| Aerosol AY | 4220 | 20.9 | " |
| TPE-STC | 1730 | 19.2 | " |
| TPME-STC | 203 | 20-9 | " |
| n=4, R=H | 15100 | 13.0 | invention |
| n=3, R=H | 14425 | 8.9 | " |
| n=2, R=H | 10130 | 18.5 | " |
| n=1, R=Me | 7555 | 17.8 | " |
| n=1, R=H | 4155 | 20.3 | comparison |

The above results show clearly that the compounds of this invention:
(i) Increase liquid dispersion reactivity as hydrophobic chain length increases. (Note: phenyl propyl is minimum chain length to give increased reactivity thus demonstrating why shorter chains such as phenylethyl lie outside the invention);
(ii) Enhance liquid dispersion reactivity relative to the aliphatic (i.e. non-phenyl ending) sulfosuccinates;
(iii) Boost liquid dispersion reactivity relative to other commonly available anionic dispersing aids, such as sodium dodecyl sulphate (SDS) and sodium dodecylbenzene sulphonate (SDBS);
(iv) Increase liquid dispersion reactivity relative to the tri-chain phenyl-ended sulphonates, such as TPE-STC (tri-2-phenylethyl sulfotricarballylate) and TPME-STC (tri-2-phenyl-2-methylethyl sulfotricarballylate) (US Patent 4,988,610), thus demonstrating that the 2 hydrophobic chain geometry of the materials of this invention is critical to their performance;
(v) Decrease particle size, especially with the longer hydrophobic chain examples of the invention, relative to other anionic surfactants, such as SDS, SDBS, aliphatic sulfosuccinates and phenyl-ended sulfotricarballylates.

### Increased Dmax

When coatings are made of the most reactive microprecipitated dispersions, the examples of the invention show the highest Dmax.

Monochrome coatings of the microprecipitated dispersions were made according to the procedures outlined.

A monochrome bilayer format was used for the photographic evaluation of the coupler dispersions:

| | | |
|---|---|---|
| Layer 2 | Gelatin | 1.614 g/m² |
| | Alkanol XC | 21.5 mg/m² |
| | BVSME | 64.0 mg/m² |
| Layer 1 | Gelatin | 1.614 g/m² |
| | Coupler VI | 0.836 mmoles/m² |
| | Silver (as chloride emulsion) | 239.0 mg/m² |
| Support | Resin-coated paper | |

The two layers were coated simultaneously.

The coatings were exposed to white light for 0.1s through a 21 step 0.15 logE increment tablet and processed in standard RA-4 chemistry. Reflection Dmax of each coating was measured using an X-Rite model 414 reflection densitometer. The results were as follows:

**TABLE VII.**

| **Coatings of Coupler VI microprecipitated dispersions.** | | |
|---|---|---|
| SURFACTANT | Dmax | Comment |
| SDS | 2.99 | comparison |
| SDBS | 2.73 | comparison |
| n=3,R=H | 3.39 | invention |
| n=2, R=H | 3.19 | invention |
| n=1, R=H | 2.71 | comparison |
| Table VII shows: (i) Dmax increases with increasing hydrophobic chain length for the materials of the invention; (ii) Higher Dmax are obtained with the longer chain length compounds of this invention than for the commonly available anionic dispersing aids such as SDS and SDBS; (iii) The advantages of higher Dmax are not seen with the short phenyl-ended sulfosuccinates which are outside the scope of this invention. | | |

### Photographic Benefits with Homogenised Oil-in-Aqueous Gelatin Dispersions of Colour Couplers

### Increased contrast and shoulder density.

Traditionally colour couplers are dissolved in a high-boiling, water-insoluble solvent and mechanically dispersed in an aqueous gelatin solution containing surfactant to facilitate dispersion. Mean droplet sizes are usually significantly larger (typically, 0.2µm) than those produced by microprecipitation techniques (typically, 0.02µm).

The homogenised dispersions were made according to the following technique:

A dispersion was made of the following general formula:

| | |
|---|---|
| Coupler VI | 11.7% |
| di-n-butylphthalate | 3.9% |
| gel | 9.5% |
| water & surfactant | 74.8% |

Coupler VI was dissolved in di-n-butyl phthalate and heated at 140°C until the coupler had completely dissolved. Gelatin was dissolved in water and heated to 70°C. Surfactant was added to the gelatin solution at a rate of 0.1 mole equivalent to coupler. The coupler solution was then added to the gelatin solution and homogenised for 3 minutes using a Kinematica Polytron set at 10,000 rpm and then passed (twice) through a Microfluidics Microfluidiser (model no. 110E) which was run at 68.95 MPa (10,000 psi) pressure and a water bath temperature of 75°C.

The coatings were made as described above and were exposed to white light for 0.1s through a 21 step 0.15 logE increment tablet and processed in standard RA-4 chemistry. The contrast, Dmax, Dmin and shoulder densities were measured using an X-Rite model 414 reflection densitometer and are shown in Table VIII

In the following Table, the comparison surfactant types are as follows:
- *Type A -*: Sulfonate
- *Type B -*: Sulfosuccinate
- *Type C -*: Sulfoitaconate having the formula
- *Type D* -: Sulfoglutaconate having the formula

**TABLE VIII.**

| **Measurements of coated dispersions of coupler VI made with different surfactants.** | | | | | |
|---|---|---|---|---|---|
| Surfactant | Contrast ±0.06 | Shoulder ±0.03 | Dmax ±0.02 | Dmin ±0.003 | Comment |
| *Type A* | 3.45 | 1.91 | 2.32 | 0.111 | comp |
| SDBS | | | | | |
| *Type B* | | | | | |
| A-OT | 3.56 | 1.94 | 2.42 | 0.110 | comp |
| n=4, R=H | 3.72 | 1.99 | 2.40 | 0.112 | inv |
| n=3, R=H | 3.77 | 2.01 | 2.51 | 0.113 | inv |
| n=2, R=H | 3.80 | 2.00 | 2.52 | | inv |
| n=1, R=Me | 3.73 | 2.00 | 2.44 | 0.113 | inv |
| n=1, R=H | 3.28 | 1.87 | 2.23 | 0.109 | comp |
| n=0, R=H | 3.39 | 1.89 | 2.36 | 0.112 | comp |
| *Type C* | | | | | |
| n=0 | 3.63 | 1.95 | 2.35 | 0.114 | comp |
| n=1 | 3.63 | 1.95 | 2.47 | 0.110 | comp |
| n=2 | 3.59 | 1.93 | 2.40 | 0.112 | comp |
| n=3 | 3.34 | 1.86 | 2.30 | 0.115 | comp |
| *Type D* | | | | | |
| n=O | 3.46 | 1.92 | 2.31 | 0.114 | comp |
| n=3 | 3.56 | 1.95 | 2.39 | 0.109 | comp |

For homogenised dispersions of coupler VI, the materials of the invention clearly show:
(i) Increased contrast and increased shoulder density relative to aliphatic, non phenyl-ended sulfosuccinates such as Aerosol OT; conventional anionic surfactants such as SDBS ω-arylalkyl phenyl-ended sulfoitaconates and sulfoglutaconates; and the shorter chain phenyl-ended sulfosuccinates which are outside the scope of this invention;
(ii) The shorter chain phenyl-ended sulfosuccinates which are outside the scope of this invention also show significantly lower Dmax emphasising the importance of chain length for the materials of this invention;
(iii) No significant Dmin penalty.
In summary, the phenyl-ended sulfosuccinate dispersing aids of this invention show advantages over a wide variety of chemically similar materials when used in the photographic context described.

### Increased liquid dispersion reactivity

Dispersions of couplers I and II were made according to the procedures shown in Example 3. The liquid dispersion measurements were made as described above and are presented in Table IX.

**Table IX.**

| **Liquid dispersion data for homogenised dispersions of couplers I and II.** | | | |
|---|---|---|---|
| Surfactant | Liquid dispersion reactivity rate constants | | Comments |
| | Coupler I | Coupler II | |
| Aerosol OT | 1820 | 12600 | comparison |
| Alkanol XC | 3920 | 10230 (±390) | comparison |
| n=2, R=H | 4690 | 19100 (±140) | invention |
| n=3, R=H | 4400 | 15800 | invention |

Table IX clearly shows that for coupler I and coupler II dispersions, the materials of the invention boost liquid dispersion reactivity relative to aliphatic, non-phenyl ended sulfosuccinates, such as Aerosol™OT, and a conventional anionic surfactant, such as Alkanol™XC.

### Example 5

### Low Foaming in Developer

Foaming can cause serious problems during photographic processing especially in seasoned developers where surfactants have leached out from the photographic product and built up in concentration. These foams can cause solution overflow, solution loss, uneven development and solution carry over into successive processing tanks.

To demonstrate that one of the preferred materials of this invention showed a lower propensity to foaming, tests were conducted with a simulated seasoned developer based on colour developer ECP-2b using the Ross-Miles foam test.

The test was first devised by Ross and Miles (Ross, J. and G D Miles, Am. Soc. for Testing Materials, Method D1173-53, Philadelphia, PA 1953; *Oil and Soap* 18, 99,1941). This test involves placing some solution in both a lower and upper reservoir; the solution passes out of the upper reservoir through a specific orifice (2.9mm i.d.), drops freely through a specified distance (initially 90 cm), then splashes into the lower reservoir. The foam so formed is measured immediately after the upper reservoir is empty, then again 5 minutes later. Foam stability is then assessed as the percentage of the height remaining after 5 minutes relative to the initial height of the foam. Obviously the lower the percentage the lower the foam stability.

To simulate seasoned developer, solutions of ECP-2b were made up at 37-38°C such that each solution contained 0.006 wt% gelatin and 0.002wt% surfactant. Each surfactant was tested independently in this format.

In the following Table, Foam Stability is defined as Foam (5min)/Foam (0min) x 100%.

**Table X.**

| **Ross-Miles Foam Tests** | | | |
|---|---|---|---|
| Surfactant | Foam (0 min) | Foam (5 min) | Foam stability |
| Comparisons | | | |
| Control (none) | 21 mm | 1 mm | 5 |
| Aerosol OT | 60 mm | 59 mm | 98 |
| Alkanol XC | 37 mm | 53 mm | 93 |
| Olin 10G | 35 mm | 31 mm | 89 |
| FT248 | 38 mm | 29 mm | 76 |
| Invention | | | |
| n=3, R=H | 37 mm | 15 mm | 41 |

Table X demonstrates that one of the preferred materials of this invention(n=3, R=1) produces significantly less foam in the simulated seasoned developer than the corresponding aliphatic sulfosuccinate, Aerosol™OT, and significantly less foam than examples of other surfactants that may be found in photographic products, e.g. Alkanol™XC, Olin 10G and FT248

## Claims

1. A method of preparing a multilayer photographic material comprises
(a) simultaneously coating on a support a plurality of aqueous hydrophilic colloid layers including at least one light-sensitive silver halide emulsion layer wherein at least one of the underlying hydrophilic colloid layers contains hydrophobic particles dispersed therein with the aid of a surfactant and,
(b) drying the coated layers, characterised in that the surfactant has the structure wherein
R is H or methyl provided that when each n=1, each R is methyl;
M is a cation; and,
n is an integer from 1 to 6;

2. Use of a surfactant having the structure wherein
R is H or methyl provided that when each n=1, each R is methyl;
M is a cation; and,
n is an integer from 1 to 6;
in the method according to claim 1 as an agent which improves coating latitude.

3. Use of a surfactant having the structure wherein
R is H or methyl provided that when each n=1, each R is methyl;
M is a cation; and,
n is an integer from 1 to 6;
in a multilayer photographic material comprising a support bearing a plurality of hydrophilic colloid layers including at least one light-sensitive silver halide emulsion layer wherein at least one of the underlying hydrophilic colloid layers contains hydrophobic particles dispersed therein with the aid of the surfactant;
in order to reduce the foaming which can occur during photographic processing of the material.

4. A method or use according to any one of claims 1 to 3 wherein the hydrophobic particles comprise a photographic coupler.

5. A method of preparing a composition comprising a hydrophilic colloid having hydrophobic particles dispersed therein comprising dispersing a hydrophobic material comprising a photographic coupler into an aqueous solution of a hydrophilic colloid in the presence of the surface active agent characterised in that the surfactant has the structure wherein
R is H or methyl provided that when each n=1, each R is methyl;
M is a cation; and,
n is an integer from 1 to 6; and,
the surfactant is used in an amount less than 1 weight percent without a washing step to remove at least one fourth of the surfactant.

6. A method or use according to any one of the preceding claims wherein each n is an integer from 2 to 4, and each R is H.

7. A method or use according to any one of the preceding claims wherein each n is 3, and each R is H.

8. A method or use according to any one of the preceding claims wherein M is an alkali metal ion.

9. A method or use according to any one of the preceding claims wherein the hydrophilic colloid is gelatin.

## Patentansprüche

1. Verfahren zur Herstellung eines mehrschichtigen photographischen Materials, bei dem man
(a) gleichzeitig auf einen Träger eine Mehrzahl von wäßrigen hydrophilen Kolloidschichten aufträgt, einschließlich mindestens einer licht-empfindlichen Silberhalogenidemulsionsschicht, wobei mindestens eine der darunter liegenden hydrophilen Kolloidschichten hierin mit Hilfe eines oberflächenaktiven Mittels dispergierte Teilchen enthält, und bei dem man
(b) die aufgetragenen Schichten trocknet,
dadurch gekennzeichnet, daß das oberflächenaktive Mittel die Struktur hat worin
R für H oder Methyl steht, wobei gilt, daß wenn jedes n=1 ist, jeder Rest R Methyl darstellt;
M ein Kation ist; und
n eine Zahl von 1 bis 6 darstellt.

2. Verwendung eines oberflächenaktiven Mittels mit der Struktur worin
R für H oder Methyl steht, wobei gilt, daß wenn jedes n=1 ist, jeder Rest R Methyl darstellt;
M ein Kation ist; und
n eine Zahl von 1 bis 6 darstellt; in dem Verfahren gemäß Anspruch 1 als Mittel, das den Beschichtungsspielraum verbessert.

3. Verwendung eines oberflächenaktiven Mittels mit der Struktur worin
R für H oder Methyl steht, wobei gilt, daß wenn jedes n=1 ist, jeder Rest R Methyl darstellt;
M ein Kation ist; und
n eine Zahl von 1 bis 6 darstellt; in einem mehrschichtigen photographischen Material mit einem Träger, auf dem sich eine Mehrzahl von hydrophilen Kolloidschichten befindet, einschließlich mindestens einer lichtempfindlichen Silberhalogenidemulsionsschicht, wobei mindestens eine der darunter liegenden hydrophilen Kolloidschichten hierin mit Hilfe des oberflächenaktiven Mittels dispergierte hydrophobe Teilchen enthält;
um das Schäumen zu vermindern, das während der photographischen Entwicklung des Materials auftreten kann.

4. Verfahren oder Verwendung nach einem der Ansprüche 1 bis 3, bei dem bzw. bei der die hydrophoben Teilchen einen photographischen Kuppler umfassen.

5. Verfahren zur Herstellung einer Zusammensetzung mit einem hydrophilen Kolloid mit hierin dispergierten hydrophoben Teilchen, bei dem man ein hydrophobes Material mit einem photographischen Kuppler in einer wäßrigen Lösung eines hydrophilen Kolloides in Gegenwart des oberflächenaktiven Mittels dispergiert, dadurch gekennzeichnet, daß das oberflächenaktive Mittel die Struktur hat worin
R für H oder Methyl steht, wobei gilt, daß wenn jedes n=1 ist, jeder Rest R Methyl darstellt;
M ein Kation ist; und
n eine Zahl von 1 bis 6 darstellt; und bei dem das oberflächenaktive Mittel in einer Menge von weniger als 1 Gew.-% verwendet wird, ohne eine Waschstufe, um mindestens ein Viertel des oberflächenaktiven Mittels zu entfernen.

6. Verfahren oder Verwendung nach einem der vorstehenden Ansprüche, wobei n jeweils für eine Zahl von 2 bis 4 steht und R jeweils H ist.

7. Verfahren oder Verwendung nach einem der vorstehenden Ansprüche, wobei n jeweils für 3 steht und R jeweils H darstellt.

8. Verfahren oder Verwendung nach einem der vorstehenden Ansprüche, wobei M ein Alkalimetallion ist.

9. Verfahren oder Verwendung nach einem der vorstehenden Ansprüche, wobei das hydrophile Kolloid Gelatine ist.

## Revendications

1. Procédé de préparation d'un produit photographique multicouche comprenant :
(a) l'application simultanée sur un support de plusieurs couches colloïdales aqueuses hydrophiles comprenant au moins une couche d'émulsion aux halogénures d'argent photosensible, dans laquelle au moins l'une des couches colloïdales hydrophiles sous-jacentes contient des particules hydrophobes dispersées à l'aide d'un agent tensio-actif et,
(b) le séchage des couches appliquées,
procédé caractérisé en ce que l'agent tensio-actif a la structure : où
R représente H ou un groupe méthyle, à condition que lorsque chaque n = 1, chaque R soit un groupe méthyle ;
M est un cation ; et,
n est un nombre entier compris entre 1 et 6.

2. Utilisation d'un agent tensio-actif ayant la structure : où
R représente H ou un groupe méthyle, à condition que lorsque chaque n = 1, chaque R soit un groupe méthyle ;
M est un cation ; et,
n est un nombre entier compris entre 1 et 6 ; dans le procédé selon la revendication 1, comme agent améliorant la latitude de couchage.

3. Utilisation d'un agent tensio-actif ayant la structure : où
R représente H ou un groupe méthyle, à condition que lorsque chaque n = 1, chaque R soit un groupe méthyle ;
M est un cation ; et,
n est un nombre entier compris entre 1 et 6 ;
dans un produit photographique multicouche comprenant un support recouvert de plusieurs couches colloïdales hydrophiles comprenant au moins une couche d'émulsion aux halogénures d'argent photosensible, dans lequel au moins l'une des couches colloïdales hydrophiles sous-jacentes contient des particules hydrophobes dispersées à l'aide de l'agent tensio-actif ;
afin de réduire le moussage qui peut se produire pendant le traitement photographique du produit.

4. Procédé ou utilisation selon l'une quelconque des revendications 1 à 3, dans lequel les particules hydrophobes comprennent un coupleur photographique.

5. Procédé de préparation d'une composition comprenant un colloïde hydrophile dans lequel sont dispersées des particules hydrophobes, comprenant la dispersion d'un matériau hydrophobe comprenant un coupleur photographique dans une solution aqueuse d'un colloïde hydrophile en présence de l'agent tensio-actif, caractérisé en ce que l'agent tensio-actif a la structure : où
R représente H ou un groupe méthyle, à condition que lorsque chaque n = 1, chaque R soit un groupe méthyle ;
M est un cation ; et,
n est un nombre entier compris entre 1 et 6 ; et l'agent tensio-actif est utilisé en une quantité inférieure à 1 pourcent en poids, sans étape de lavage pour éliminer au moins un quart de l'agent tensio-actif.

6. Procédé ou utilisation selon l'une quelconque des revendications précédentes, dans lequel chaque n est un nombre entier compris entre 2 et 4, et chaque R représente H.

7. Procédé ou utilisation selon l'une quelconque des revendications précédentes, dans lequel chaque n est égal à 3 et chaque R représente H.

8. Procédé ou utilisation selon l'une quelconque des revendications précédentes, dans lequel M représente un ion de métal alcalin.

9. Procédé ou utilisation selon l'une quelconque des revendications précédentes, dans lequel le colloïde hydrophile est de la gélatine.
